

# UNITED STATES PATENT OFFICE.

LOUIS SCHULTE, OF PITTSBURGH, PENNSYLVANIA, ASSIGNOR TO E. I. DU PONT DE NEMOURS & COMPANY, OF WILMINGTON, DELAWARE, A CORPORATION OF DELAWARE.

## NICKEL-PLATING SOLUTION.

1,379,050.

Specification of Letters Patent. Patented May 24, 1921.

No Drawing.

Application filed July 24, 1918. Serial No. 246,531.

To all whom it may concern:

Be it known that I, LOUIS SCHULTE, of Pittsburgh, in the county of Allegheny and in the State of Pennsylvania, have invented a certain new and useful Improvement in Nickel-Plating Solutions, and do hereby declare that the following is a full, clear, and exact description thereof.

The object of my invention is to provide a solution suitable for the electro-deposition of nickel plate, which solution, although capable of general application, is particularly adapted for depositing nickel upon a highly polished nickel surface.

15 A further object of the invention is to provide such a solution which will produce a soft, bright and flexible nickel coating, and by means of which the plating operation may be carried out in a relatively short time, 20 and having high current activity.

Further objects and advantages of the invention will be in part obvious and in part specifically mentioned in the description contained hereinafter, in which I have 25 disclosed one embodiment of my invention, which embodiment however, is to be considered merely as illustrative of its principle.

I have found it to be advantageous to 30 employ an alkali salt, such as sulfate of sodium in combination with the nickel containing ingredients of the solution, inasmuch as the sodium salt gives a good conductivity to the solution, thus enabling a 35 higher current to be used, and the plating process to be carried out in a shorter time. The sodium salt also aids in the production of a flexible nickel deposit having a bright surface.

40 The sodium salt is combined in the solution with nickel salts, preferably sulfate of nickel, and a certain amount of double sulfate of nickel and ammonia. It is also advantageous to acidify the bath or solution 45 to some extent by the addition of a weak acid, such as acetic acid.

I prefer to make up the solution by com-

bining the above elements in approximately the proportions stated below:

|                                           |       |    |
|-------------------------------------------|-------|----|
| Sulfate of nickel-----                    | 17%   | 50 |
| Double sulfate of nickel and ammonia----- | 1.4%  |    |
| Sulfate of sodium-----                    | 8.5%  |    |
| Acetic acid-----                          | 2.2%  |    |
| Water-----                                | 70.9% | 55 |

The proportions of the ingredients however may be varied to a considerable extent without producing any detrimental effect in the nickel deposit.

60 A solution of the character above described will deposit nickel uniformly upon another nickel surface even though said surface be highly polished, and the deposit is substantially without peeling or blistering, 65 and still is soft and bright. Such a solution is particularly useful in plating nickel upon nickel, for instance in the process of renovating press polishing plates, as described in my co-pending application, Serial Number 246,532, filed July 24, 1918.

70 I claim:

1. A nickel plating solution containing sulfate of sodium and single and double nickel salts. 75
2. A nickel plating solution containing sulfate of sodium, nickel sulfate, and double sulfate of nickel and ammonia.
3. A nickel plating solution containing approximately 8% sulfate of sodium, and 80 15-20% sulfate of nickel.
4. A nickel plating solution containing approximately 8% sulfate of sodium, 15-20% sulfate of nickel, and a relatively small percentage of double sulfate of nickel and ammonia. 85
5. A nickel plating solution containing sulfate of sodium, single and double nickel salts, and a weak acid.
6. A nickel plating solution containing 90 sulfate of sodium, nickel sulfate, double sulfate of nickel and ammonia, and a weak acid.
7. A nickel plating solution containing

- approximately 8% sulfate of sodium, 15-20% sulfate of nickel, and a weak acid.
8. A nickel plating solution containing approximately 8% sulfate of sodium, 5 15-20% sulfate of nickel, a relatively small percentage of double sulfate of nickel and ammonia, and a weak acid.
9. A nickel plating solution containing sulfate of sodium, single and double nickel 10 salts, and acetic acid.
10. A nickel plating solution containing sulfate of sodium, nickel sulfate, double sulfate of nickel and ammonia, and acetic acid.
11. A nickel plating solution containing approximately 8% sulfate of sodium, 15-20% sulfate of nickel, and about 2% of acetic acid.
12. A nickel plating solution containing approximately 8% sulfate of sodium, 15-20% sulfate of nickel, a relatively small 20 percentage of double sulfate of nickel and ammonia, and about 2% of acetic acid.

In testimony that I claim the foregoing I have hereunto set my hand.

LOUIS SCHULTE.